



were irregular and particularly dull within the medium and high current density range.

The sulfonic acid salt was obtained by admixing 12.9 parts by weight caprothiolactam with 21.1 parts by weight bromoethane-sodium sulfonate, adding 50 parts by weight of water and heating the mixture for a short period of time to about 105-110° C. until a clear solution was formed. Upon cooling, the sodium salt of isocaprothiolactam-S-ethyl ester- $\omega$ -sulfonic acid precipitated out in the form of yellow crystals with a yield of 13-15 parts by weight (=50-58% of theory).

*Example III*

A cyanide cadmium bath, containing 70 gm./liter cadmium cyanide, 50 gm./liter sodium cyanide and 30 gm./liter sodium hydroxide, was modified with 2.5 gm./liter of the internal salt of isocaprothiolactam-S-n-propyl ester- $\omega$ -sulfonic acid as a brightening agent. The cadmium electrodeposited at room temperature and at current densities between 2 and 6 amp./dm.<sup>2</sup> on sheet iron formed a full-bright, ductile plate.

The brightening agent used above was obtained by heating a mixture of 2.58 parts by weight caprothiolactam and 2.45 parts by weight propane sultone to 60° C. The temperature rose rapidly to 140 to 160° C. Upon cooling, the solidified melt thus obtained was dissolved in glacial acetic acid, the solution was concentrated slightly and was then triturated with ethyl acetate and acetone, whereby the internal salt of isocaprothiolactam-S-n-propyl ester- $\omega$ -sulfonic acid crystallized out as a grainy, faintly yellow substance. After washing the product with acetone and drying it, the salt was obtained with a yield of 4.1 parts by weight (79% of theory). After recrystallization from glacial acetic acid it melted at 257° C. (uncorrected).

*Example IV*

Sheet steel was electroplated at room temperature and at a current density of 2-5 amp./dm.<sup>2</sup> in an acid zinc bath which contained 240 gm./liter zinc sulfate, 5 gm./liter sodium acetate, 5 gm./liter boric acid and as a brightening agent 3 gm./liter of the sodium salt of 4-S- $\Delta'$ -piperideinyl-(2')-mercapto - butane - sulfonic acid-1. The zinc electrodeposits thus obtained were full-bright.

While we have set forth specific embodiments and preferred modes of practice of our invention, it will be understood that the invention is not limited to these embodiments and that various changes and modifications may be made without departing from the spirit of the disclosure and the scope of the appended claims.

We claim:

1. An electroplating bath for producing bright electrodeposits of metals selected from the group consisting of copper, zinc, cadmium, tin, brass, bronze, silver and gold, comprising a solution of a salt of the metal to be deposited and as a brightening agent a water soluble sulfonic acid of the general formula



and water soluble salts thereof, wherein R represents a polymethylene chain and R<sub>1</sub> represents a bivalent hydrocarbon radical, said brightening agent being present in sufficient amount to obtain said bright electrodeposits.

2. The bath of claim 1 wherein the R polymethylene chain of the brightening agent is a substituted polymethylene chain.

3. The bath of claim 1 wherein the R<sub>1</sub> bivalent hydrocarbon radical of the brightening agent has substituents selected from the group consisting of hydroxyl groups and halogen atoms.

4. The bath of claim 1 comprising in addition a compound selected from the group consisting of thioamides

and isothioamides, said compound being free of sulfonic acid groups.

5. The bath of claim 1 wherein the bath is an acid bath.

6. The bath of claim 1 wherein the bath is an alkaline bath.

7. The bath of claim 1 wherein the bath is a cyanide bath.

8. An electroplating bath for producing bright electrodeposits of metals selected from the group consisting of copper, zinc, cadmium, tin, brass, bronze, silver and gold, comprising a solution of a salt of the metal to be deposited and as a brightening agent 0.01 to 10 gm./liter of a water soluble sulfonic acid of the general formula



and water soluble salts thereof, wherein R represents a polymethylene chain and R<sub>1</sub> represents a bivalent hydrocarbon radical.

9. The bath of claim 8 wherein the brightening agent is the sodium salt of isocaprothiolactam-S-hydroxy-25 propyl-ester-1'-sulfonic acid.

10. The bath of claim 8 wherein the brightening agent is the sodium salt of isocaprothiolactam-S-ethyl ester- $\omega$ -sulfonic acid.

11. The bath of claim 8 wherein the brightening agent is the sodium salt of 4-S- $\Delta'$ -piperideinyl-(2')-mercapto-butane-sulfonic acid-1.

12. A process for producing bright electrodeposits of metals selected from the group consisting of copper, zinc, cadmium, tin, brass, bronze, silver and gold, which comprises depositing said metal from an electroplating bath containing the metal to be deposited in the form of a salt in the presence of a brightening agent comprising a water soluble sulfonic acid of the general formula



and water soluble salts thereof, wherein R represents a polymethylene chain and R<sub>1</sub> represents a bivalent hydrocarbon radical, said brightening agent being present in sufficient quantity to effect said brightening.

13. The process of claim 12 wherein the R polymethylene chain of the brightening agent is a substituted polymethylene chain.

14. The process of claim 12 wherein the R<sub>1</sub> bivalent hydrocarbon radical of the brightening agent has substituents selected from the group consisting of hydroxyl groups and halogen atoms.

15. The process of claim 12 wherein the bath contains in addition a compound selected from the group consisting of thioamides and isothioamides, said compound being free of sulfonic acid groups.

16. A process for producing bright electrodeposits of metals selected from the group consisting of copper, zinc, cadmium, tin, brass, bronze, silver and gold, which comprises depositing said metal from an electroplating bath containing the metal to be deposited in the form of a salt in the presence of 0.01 to 10 gm./liter of a brightening agent comprising a water soluble sulfonic acid of the general formula



and water soluble salts thereof, wherein R represents a polymethylene chain and R<sub>1</sub> represents a bivalent hydrocarbon radical.

17. The process of claim 16 wherein the brightening

agent is the sodium salt of isocaprothiolactam-S-hydroxy-propyl-ester-1'-sulfonic acid.

18. The process of claim 16 wherein the brightening agent is the sodium salt of isocaprothiolactam-S-ethyl ester- $\omega$ -sulfonic acid.

19. The process of claim 16 wherein the brightening agent is the sodium salt of 4-S- $\Delta'$ -piperideinyl-(2')-mercapto-butane-sulfonic acid-1.

References Cited in the file of this patent

UNITED STATES PATENTS

|           |                         |               |
|-----------|-------------------------|---------------|
| 2,489,538 | Phillips et al. -----   | Nov. 29, 1949 |
| 2,663,684 | Pierce -----            | Dec. 22, 1953 |
| 2,830,014 | Gundel et al. -----     | Apr. 8, 1958  |
| 2,849,351 | Gundel et al. -----     | Aug. 26, 1958 |
| 2,849,352 | Kirstahler et al. ----- | Aug. 26, 1958 |

UNITED STATES PATENT OFFICE  
CERTIFICATE OF CORRECTION

Patent No. 3,023,150

February 27, 1962

Wolf-Dieter Willmund et al.

It is hereby certified that error appears in the above numbered patent requiring correction and that the said Letters Patent should read as corrected below.

Column 2, line 19, for "typing" read -- tying --; line 26, for "of iron" read -- on iron --.

Signed and sealed this 7th day of August 1962.

(SEAL)

Attest:

ERNEST W. SWIDER  
Attesting Officer

DAVID L. LADD  
Commissioner of Patents